

## UNITED STATES PATENT OFFICE

2,313,162

## TREATMENT OF HYDROCARBONS

Jacque C. Morrell and Aristid V. Grosse, Chicago,  
Ill., assignors to Universal Oil Products Com-  
pany, Chicago, Ill., a corporation of Delaware

No Drawing. Application March 25, 1939,  
Serial No. 264,207

14 Claims. (Cl. 260—683)

This invention relates particularly to the treatment of aliphatic or straight chain hydrocarbons which are either completely saturated, as in the case of the paraffinic hydrocarbons, or straight chain hydrocarbons which may be unsaturated to the extent of their possessing one double bond between carbon atoms, as in the case of the mono-olefinic hydrocarbons. The invention is directed primarily to the treatment of aliphatic hydrocarbons having less than 6 carbon atoms in straight chain arrangement, including ethane, ethylene, propane, propylene, butanes, butylenes, pentanes, and amylenes, although it may also be applied to hydrocarbons of more than six carbon atoms. The present application is a continuation-in-part of our earlier application Serial No. 105,714, filed October 15, 1936.

In a more specific sense the invention is concerned with a new and improved type of process for controllably increasing the degree of unsaturation in hydrocarbons of the character mentioned so that, for example, a paraffin hydrocarbon may be converted either into its corresponding mono-olefin or di-olefin or a mono-olefinic hydrocarbon may be converted into a diolefin with a practical minimum of undesirable side reactions.

The present process is concerned with the more efficient utilization of aliphatic hydrocarbons of the types mentioned above in that they are converted by dehydrogenation into compounds of a more reactive character which are readily utilisable in the production of polymers and miscellaneous hydrocarbon derivatives useful in the arts.

In the complete utilization of petroleum to form maximum yields of automotive fuel there is a considerable production of gaseous paraffinic hydrocarbons which are dissolved in the crude oils as produced and evolved as a light cut in the production of straight run gasoline and there are further quantities of similar paraffinic gases produced in connection with the natural gas and natural gasoline industries. These gases are too volatile for direct utilization as motor fuel except in special instances and at the present time their principal use is as domestic fuel. Owing to their generally unreactive character, it is difficult to transform them into increased yields of motor fuel unless they are converted into their corresponding olefinic counterparts by splitting off a molecule of hydrogen. After this is done the resulting olefins may be polymerized either by heat alone or by heat and catalysts to form gasoline boiling range polymers which are of high anti-knock value and eminently suitable as blending

fluid for increasing the knock-rating of straight run gasolines which are usually inferior in this respect.

In applying the present invention to the manufacture of mono-olefins from normally gaseous paraffins, the invention is related to processes involving the more complete utilization of the gases produced in connection with the production and refining of petroleum since the olefinic gases are readily polymerizable by various thermal and catalytic methods to produce liquid polymers having a relatively high octane rating and boiling within the range of gasoline and which may be either utilized as such or hydrogenated to corresponding liquid paraffins. Thus according to the present process the residual paraffins remaining after the olefins primarily present in cracked gas mixtures have been polymerized, may be subjected to the treatment to produce additional quantities of polymerizable olefins.

In the process for manufacturing diolefins either from paraffins or mono-olefins according to the present process the invention is related to the synthetic rubber problem in that butadienes and their alkylated derivatives are producible from 4 and 5 carbon atom aliphatic hydrocarbons and these butadienes are polymerizable to form high molecular weight polymers closely resembling natural rubber.

In experimenting with methods and conditions for converting paraffin hydrocarbons into olefins by dehydrogenation, a considerable number of catalytic materials have been tried with greater or lesser effectiveness, since it has been found generally that better results in the matter of yield of olefins without the formation of liquid and gaseous by-products are obtainable by the use of catalysts rather than by the use of heat alone, and furthermore that under proper catalytic influences temperatures, pressures, and time factors are lower, so that less expensive apparatus may be employed and greater capacities insured.

In one specific embodiment the present invention comprises the treatment of paraffinic or mono-olefinic hydrocarbons for the dehydrogenation thereof by subjecting said hydrocarbons at temperatures of the order of 450-700° C. and relatively low pressures to contact with solid-granular catalysts consisting essentially of aluminum oxide mixed with or supporting oxides of the elements in the left-hand column of group V of the periodic table, which oxides have been found to have relatively high catalytic activity in furthering straight dehydrogenation reactions.

The present invention is characterized by the use of particular catalytic materials and suitable combinations of temperature, pressure, and time of contact to control the character and extent of the dehydrogenation of aliphatic hydrocarbons to produce a minimum of undesirable by-products. Temperatures from approximately 450 to 700° C. may be employed, pressures from moderately superatmospheric of the order of 50 to 100 lbs. per square inch down to those of the order of 0.25 atmosphere absolute or lower and times of contact from approximately 0.01 to 10 seconds. In the case of the dehydrogenation of paraffinic hydrocarbons to produce the corresponding mono-olefins, temperatures within the approximate range of 450 to 650 may be employed, atmospheric pressures and times of contact of the order of 0.1 to 6 seconds. When producing diolefins from mono-olefins, temperatures from 500 to 700° C. are preferred, absolute pressures of approximately 0.25 atmosphere and times of contact of less than 1 second. When it is desired to produce diolefins directly from paraffins without a primary stage involving the production and segregation of the mono-olefins, intermediate conditions of operation may be employed which will be more or less fixed by the molecular weight and constituents of the paraffin or mixture of paraffins to be subjected to treatment.

In accordance with the present invention, the catalysts which are preferred for selectively dehydrogenating aliphatic hydrocarbons have been evolved as the result of a large amount of investigation with catalysts having a dehydrogenating action upon various types of hydrocarbons such as, for example, those which are encountered in the fractions produced in the distillation and/or pyrolysis of petroleum and other naturally occurring hydrocarbon oil mixtures. The criterion of an acceptable dehydrogenating catalyst is that it shall split off hydrogen without inducing either scission of the bonds between carbon atoms or carbon separation.

It should be emphasized that in the field of catalysts there have been very few rules evolved which would enable the prediction of what materials will catalyze a given reaction. Most of the catalytic work has been done on a purely empirical basis, though at times certain groups of elements or compounds have been found to be more or less equivalent in accelerating certain types of reaction. For example, the noble metals, platinum and palladium, have been found to be effective in dehydrogenating reactions, particularly in dehydrogenating naphthalenes to form aromatics, but these metals are expensive and easily poisoned by traces of sulfur so that their use is considerably limited in petroleum hydrocarbon reactions.

The present invention is characterized by the use of a particular group of composite catalytic materials which contain aluminum oxide which in itself has some catalytic ability in the dehydrogenating reactions but which is improved greatly in this respect by the addition to or admixture therewith of certain other catalysts (most generally in minor proportions), which comprise in the present instance the oxides of the elements in the left-hand column of group V of the periodic table which include vanadium, columbium, and tantalum.

It is essential to the preparation of these active and selective dehydrogenative catalysts that the aluminum oxide used possess certain struc-

tural characteristics permitting the maintenance on its surface and in its pores of a stable deposit of the more active oxide catalysts which is essentially undisturbed under the conditions of operation and when regenerating by burning off carbonaceous deposits with air or other oxygen-containing gas mixtures.

The more active compounds or promoters which are used in the catalyst composites according to the concepts of the present invention include the oxides of vanadium, columbium and tantalum which constitute a natural group since they are the elements in the left-hand column of group V of the periodic table. While the oxides of these elements are effective catalysts in the dehydrogenation reactions, it is not intended to infer that the different oxides of any one element or the corresponding oxides of the different elements are exact equivalents in their catalytic activity.

Catalyst composites may be prepared by utilizing the soluble compounds of the elements containing a volatile radical in aqueous solutions from which they are absorbed by the prepared alumina or from which they are deposited upon the alumina by evaporation of the solvent, after which the volatile radical is driven off by heat. The invention further comprises the use of catalyst composites made by mixing compounds of the above-mentioned character or prepared oxides with the alumina either in the wet, dry or fused condition. In the following paragraphs some of the compounds of the elements listed above are given which may be used to add the catalytic oxides to the alumina. The known oxides of these elements are also listed.

#### VANADIUM

Catalysts comprising alumina and up to 25 per cent by weight of the lower oxides of vanadium such as the sesquioxide  $V_2O_3$  and the tetroxide  $V_2O_4$  may be effectively used. Some of the monoxide  $VO$  may be present in some instances. Thus solutions of the ammonium vanadate may be employed to add vanadium oxides to the alumina and also the soluble vanadyl sulfates and the vanadium nitrate and carbonate. The oxides per se or those produced by reduction or decomposition of other vanadium compounds may be used.

#### COLUMBIUM

A properly prepared alumina may be ground and sized to produce granules of relatively small mesh of the approximate order of from 4 to 20 and these caused to absorb compounds which will ultimately yield oxides of columbium on heating to a proper temperature by stirring them with warm aqueous solutions of soluble columbium compounds. The oxide resulting from the decomposition of such compounds as the pentahydroxide is for the most part the pentoxide  $Cb_2O_5$ . This oxide, however, is reduced to a definite extent by hydrogen or by the gases and vaporous products resulting from the decomposition of the paraffins treated in the first stages of the process, so that the essential catalysts for the larger portion of the period of service are evidently the lower oxides  $CbO_2$ ,  $Cb_2O_3$ , and  $CbO$ .

#### TANTALUM

Compounds of tantalum, such as for example, the pentoxide  $Ta_2O_5$  and the tetroxide  $Ta_2O_4$ , and possibly the sesquioxide  $Ta_2O_3$ , which result from the reduction of the pentoxide and par-

ticularly efficient as catalysts for the present types of reactions. Tantulum fluoride is soluble in water and may be conveniently used in aqueous solution as a source of the oxides which result from the ignition of the precipitated hydroxide to form the pentoxide, the partial reduction of this oxide by hydrogen or the gases and vapors in contact with the catalyst in the normal operation of the process forming the desired lower oxides. The tantalum pentahydroxide may be precipitated from a solution of the fluoride by the use of ammonium or alkali metal hydroxides or carbonates as precipitants, the hydroxide being later ignited to form the pentoxide, which may undergo some reduction as already stated.

Aluminum oxides prepared by careful calcination of certain natural hydroxides and carbonates and by carefully regulated chemical precipitation of aluminum hydroxide followed by calcination are practically always good supporting materials for the preferred dehydrogenating oxides in accordance with the present invention. While some forms of alumina may have in themselves some slight dehydrogenating activity, an extensive series of experiments has definitely shown that any inherent catalytic property which different forms of prepared alumina may have may be greatly increased by the addition of oxides of the present character in amounts usually of the order of less than 25% of the total composite of alumina and the oxide.

Aluminum oxide suitable as the base material for the manufacture of catalysts for the process may be obtained from some natural aluminum oxide minerals or ores such as bauxite or carbonates such as dawsonite by proper calcination, prepared by precipitation of aluminum hydroxide from solutions of aluminum sulfate, nitrate, chloride, or different other salts, and dehydration of the precipitate of aluminum hydroxide by heat. Usually it is desirable and advantageous to further treat it with air or other gases, or by other means to activate it prior to use.

Three hydrated oxides of aluminum occur in nature, to wit, hydrargillite or gibbsite having the formula  $Al_2O_3 \cdot 3H_2O$ , bauxite having the formula  $Al_2O_3 \cdot 2H_2O$ , and diasporite having the formula  $Al_2O_3 \cdot H_2O$ . Of these three minerals the corresponding oxides from the trihydrated and dihydrated minerals are suitable for the manufacture of alumina for the present type of catalysts and these materials have furnished types of activated alumina which are entirely satisfactory. Precipitated trihydrates can also be dehydrated at moderately elevated temperatures to form satisfactory alumina supports.

It is best practice in the final steps of preparing substantially anhydrous aluminum oxides for use in the catalyst composites to ignite them for some time at temperatures within the approximate range of from 800-900° C. This does not correspond to complete dehydration of the hydrated oxides but gives catalytic materials of good strength and porosity so that they are able to resist for a long period of time the deteriorating effects of the service and regeneration periods to which they are subjected.

While other forms of aluminum oxide may be used, it is of considerable advantage to employ the type of aluminum oxide known as gamma-alumina, by which is meant the modification obtained by the dehydration of the monohydrate termed böhmite ( $AlO(OH)$ ) or the trihydrate

$Al(OH)_3$ , termed hydrargillite (or gibbsite, when occurring in nature), at temperatures above 250° C. and preferably of the order of 350-500° C. until a substantial equilibrium is established corresponding to the removal of substantially all of the water and the formation of crystals falling within the regular or cubic classification. Gamma-alumina is characterized by definite crystallographic properties and can be readily distinguished from the large number of other modifications of alumina, such as alpha, beta, epsilon, zeta, etc., by its X-ray diffraction pattern. The gamma-alumina crystallizes in the cubic system with the edge of the unit cube being about 7.9 Angstrom units.

The most general method for adding the more active oxides to the prepared activated alumina, which has a high adsorptive capacity, is to stir the prepared granules of from approximately 4 to 20 mesh into solutions of salts which will yield the desired promoting oxides on ignition under suitable conditions. In some instances the granules may be merely stirred in slightly warm solutions of salts until the dissolved compounds have been retained on the particles by absorption or occlusion, after which the particles are separated from the excess solvent by settling or filtration, washed with water to remove excess solution, and then ignited to produce the desired residual oxide. In cases of certain compounds of relatively low solubility it may be necessary to add the solution in successive portions to the alumina with intermediate heating to drive off solvent in order to get the required quantity of oxide deposited upon the surface and in the pores of the alumina. The temperatures used for drying and calcining after the addition of the promoters from solutions will depend entirely upon the individual characteristics of the compound added and no general ranges of temperatures can be given for this step.

In some instances promoters may be deposited from solutions by the addition of precipitants which cause the deposition of dissolved materials upon the alumina granules. As a rule methods of mechanical mixing are not preferable, though in some instances as in the case of hydrated or readily fusible compounds these may be mixed with the proper proportions of alumina and uniformly distributed during the condition of fusing or fluxing.

Catalysts composites may be made by mixing alumina powders with the preferred oxides, by depositing hydroxides upon alumina powders suspended in solutions of the salts of the preferred metals, by absorbing aqueous acids or nitrates upon alumina powder or by co-precipitation of aluminum hydroxide and metal hydroxides, after which the dried and powdered materials are pelleted in any standard type of machine. Any obvious procedure necessary to obtain a pellet of uniform characteristics may be employed and any minor amount of lubricant may be used which is effective in preventing sticking or abrasion of the parts of the machine used.

In regard to the relative proportions of alumina and promoting oxides it may be stated in general that the latter are generally less than 25% by weight of the total composites, as these percentages usually give the best results from an activity and life standpoint, when considering all economic features. The effect upon the catalytic activity of the alumina caused by varying the percentage of any given oxide or mix-

ture of oxides deposited thereon is not a matter for exact calculation but more one for determination by experiment. Frequently good increases in catalytic effectiveness are obtainable by the deposition of as low as 1% to 5% of an oxide upon the surface and in the pores of the alumina, though the general average is about 15-20%.

In practicing the dehydrogenation of aliphatic hydrocarbons according to the present process a solid composite catalyst prepared according to the foregoing alternative methods is used as filler in a reaction tube or chamber in the form of particles of graded size or small pellets and the hydrocarbon gas or vapor to be dehydrogenated is passed through the catalyst after being heated to the proper temperature, under a definite pressure and for a time of contact adapted to produce the results desired. The catalyst tube may be heated exteriorly if desired to maintain the proper reaction temperature.

As an alternative and frequently preferable method of operation with the present types of catalysts, they may be used as refractory filling material in the form of bricks or special forms or as a coating upon bricks or other forms in furnaces of the regenerative type which are alternately blasted and then used as heating means to effect the desired conversion reactions. In such an operation a regenerative chamber may be filled with alternate layers of ordinary non-catalytic refractory forms and layers of catalytic materials. In this method of operation the heat necessary for the dehydrogenation reactions is added during the regenerating period which must be employed in any event to periodically remove carbonaceous deposits from the catalyst surfaces.

It has been found essential to the efficient and selective dehydrogenation of aliphatic hydrocarbons when using the present types of catalysts that the gaseous or vaporized materials be substantially free from water vapor. If appreciable amounts of steam are present, the catalytic activity is adversely affected so that the active life is shortened, the need for regeneration becomes more frequent and a point is more quickly reached where regeneration is no longer effective. The reasons for this phenomenon are not entirely clear but may possibly be due to a certain degree of hydration of the more active catalytic components of the mixtures or the hydration of the aluminum oxide support.

The exit gases from the tube or chamber may be passed through selective absorbents to combine with or absorb the unsaturated hydrocarbons produced. Mono-olefins may be selectively polymerized by suitable catalysts, caused to alkylate other hydrocarbons such as aromatics or treated directly with chemical reagents to produce desirable and commercially valuable derivatives. Di-olefins or di-olefin derivatives may be catalytically condensed or polymerized to form synthetic rubber products as already mentioned. After the olefins have been removed the residual gases may be recycled for further dehydrogenating treatment with or without removal of hydrogen.

Members of the present group of catalysts are selective in removing two hydrogen atoms from aliphatic hydrocarbon molecules to produce the corresponding straight-chain unsaturated products without furthering to any great degree undesirable side reactions, and because of this show

an unusually long period of activity in service as will be shown in later examples. When, however, their activity begins to diminish it is readily regenerated by the simple expedient of oxidizing with air or other oxidizing gas at a moderately elevated temperature, usually within the range employed in the dehydrogenating reactions. This oxidation effectively removes traces of carbon deposits which contaminate the surface of the particles and decrease their efficiency. It is characteristic of the present types of catalysts that they may be repeatedly regenerated without material loss of porosity or catalyzing efficiency.

The following examples are given to indicate the selective character of the dehydrogenation reactions produced by catalysts comprised within the present group, though they are merely selected from a large number and not given with the intent of unduly limiting the scope of the invention.

#### EXAMPLE I

The catalyst was prepared by dissolving 16 parts by weight of ammonium metavanadate in 200 parts by weight of hot water and adding the solution in two equal successive portions to 200 parts by weight of a 10-12 mesh activated alumina. After the addition of the first half of the solution the particles were somewhat damp and were dried at a steam temperature to remove excess water. After the heating, the second half of the solution was added and the dehydration repeated. During the heating period ammonia and water were evolved leaving vanadium pentoxide deposited on the alumina particles.

In this case a mixture of paraffinic gases constituting the residue after the polymerization of the olefins in a cracked gas mixture was the starting material. This gas consisted of 10% propane, 45% n-butane, and 45% isobutane. The gas mixture was passed over the catalyst at atmospheric pressure and a temperature of 500° C.

The following table shows the composition of the outlet gases at different times in the run.

#### Composition of exit gases

|                          |    |    |     |
|--------------------------|----|----|-----|
| Time after start, hours  | 22 | 72 | 120 |
| 1-Butylene               | 13 | 15 | 17  |
| Propylene and n-butylens | 7  | 10 | 8   |
| Ethylene                 | 1  | 1  | 1.5 |
| Total higher olefins     | 20 | 25 | 25  |
| Hydrogen                 | 30 | 27 | —   |

An examination of the above data indicates the high degree of selectivity of the present type of catalyst, since the percentage by volume of hydrogen is approximately equivalent to the production of higher olefins, and there is a very small percentage of ethylene present.

#### EXAMPLE II

Owing to the relative insolubility of most of the compounds of tantalum the method of dry mechanical mixing was resorted to in making up a catalyst thus one part by weight of tantalum dioxide was mixed with about 10 parts by weight of activated alumina which had been produced by calcining bauxite at a temperature of about 700° C., followed by grinding and sizing to produce particles of approximately 8-12 mesh. The catalyst particles were not treated with hydrogen on account of the known difficulty in reducing tantalum oxide although some reduction evidently took place when the hydrocarbon gas was

passed over the mass in the first stages of the treatment.

Pure propane was passed over this catalyst at atmospheric pressure and 600° C. with contact times of 1 to 2 seconds, the composition of the exit gases obtained during a run being shown below:

|           | Per cent |
|-----------|----------|
| Propylene | 24       |
| Hydrogen  | 25       |
| Methane   | 1.0      |
| Propane   | 50       |
| Ethylene  | 0.5      |

This gas composition was substantially unchanged after three successive regenerations.

#### EXAMPLE III

A catalyst was prepared by dissolving 15.4 parts by weight of ammonium metavanadate in 200 parts by weight of hot water and adding the solution in two equal successive portions to 200 parts by weight of a 10 to 12 mesh activated alumina. After the addition of the first half of the solution the particles were somewhat damp and were dried at a steam temperature to remove excess water. After this heating the second half of the solution was added and the dehydration repeated. During the heating period ammonia and water were evolved leaving vanadium pentoxide deposited on the alumina particles.

The final steps in the preparation of the catalyst comprised heating at 200-250° C. for several hours, adding the particles to a catalyst chamber in which they were brought up to the necessary reaction temperature for dehydrogenating a mono-olefinic gas mixture in a current of air, and then subjecting them to the action of hydrogen at the operating temperature to produce the lower oxides, this change being accompanied by change in color from yellow to bluish gray.

Using the catalyst prepared in the above manner a mixture of approximately equal parts of alpha and beta butylenes was dehydrogenated at a temperature of 610° C., a pressure of 0.25 atmosphere and a contact time of 0.7 second. In the products which were condensed by cooling at -80° C., 1,3-butadiene was found to be present in a concentration of about 37 per cent, corresponding to a yield of about 21 per cent based on the materials charged. The identification was made by means of the reaction with maleic anhydride, and further identification was made by the formation of the compound: 1,2,3,4-tetrabromobutane.

#### EXAMPLE IV

A catalyst was prepared for use in dehydrogenation of mixtures of alpha and beta butenes as representing mono-olefins. Owing to the relative insolubility of most of the compounds of tantalum the method of dry mechanical mixing was resorted to in making up a catalyst. Thus three parts by weight of tantalum dioxide was mixed with about 15 parts by weight of activated alumina which had been produced by calcining bauxite at a temperature of about 700° C., followed by grinding and sizing to produce particles of approximately 8-12 mesh. The catalyst particles were not treated with hydrogen on account of the known difficulty in reducing tantalum oxide although some reduction evidently took place when the hydrocarbon gas was passed over the mass in the first stages of the treatment.

Using the catalyst prepared in the above man-

ner a mixture of approximately equal parts of alpha and beta butylenes was dehydrogenated at a temperature of 615° C., a pressure of 0.25 atmosphere and a contact time of 0.80 second. In the products which were condensed by cooling at -80° C., 1,3-butadiene was found to be present in a concentration of about 36 per cent, corresponding to a yield of about 22 per cent based on the materials charged. The identification was made by means of the reaction with maleic anhydride, and further identification was made by the formation of the compound: 1,2,3,4-tetrabromobutane.

The foregoing specification and examples show clearly the character of the invention and the results to be expected in its application to aliphatic hydrocarbons, although neither section is intended to be unduly limiting.

We claim as our invention:

- 20 1. A process for the dehydrogenation of aliphatic hydrocarbons having less than six carbon atoms in straight chain arrangement to produce unsaturated derivatives thereof, which comprises subjecting said aliphatic hydrocarbons at a temperature of the order of 450-700° C., absolute pressure of the order of 0.25 to 7 atmospheres, and time from approximately 0.1 to 10 seconds to contact with a solid granular catalyst comprising essentially aluminum oxide which has a relatively low catalytic activity supporting an oxide which has a relatively high catalytic activity selected from the group consisting of the oxides of vanadium, columbium and tantalum.
- 25 35 2. A process for the dehydrogenation of aliphatic hydrocarbons to produce unsaturated derivatives thereof, which comprises subjecting said aliphatic hydrocarbons at a temperature of the order of 450-700° C., absolute pressure of the order of 0.25 to 7 atmospheres, and time from approximately 0.1 to 10 seconds to contact with a solid granular catalyst comprising essentially activated aluminum oxide which has a relatively low catalytic activity supporting an oxide which has a relatively high catalytic activity selected from the group consisting of the oxides of vanadium, columbium, and tantalum.
- 30 40 45 55 60 65 70 75 80 85 90 95 100 110 120 130 140 150 160 170 180 190 200 210 220 230 240 250 260 270 280 290 300 310 320 330 340 350 360 370 380 390 400 410 420 430 440 450 460 470 480 490 500 510 520 530 540 550 560 570 580 590 600 610 620 630 640 650 660 670 680 690 700 710 720 730 740 750 760 770 780 790 800 810 820 830 840 850 860 870 880 890 900 910 920 930 940 950 960 970
3. A process for the dehydrogenation of paraffin hydrocarbons to produce diolefins therefrom, which comprises subjecting said paraffin hydrocarbons at a temperature of the order of 500-700° C. subatmospheric pressure and time of the order of 0.01 to 2 seconds to contact with a solid granular catalyst comprising essentially aluminum oxide which has relatively high catalytic activity selected from the group consisting of the oxides of vanadium, columbium and tantalum.
4. A process for the dehydrogenation of paraffin hydrocarbons to produce diolefins therefrom, which comprises subjecting said paraffin hydrocarbons at a temperature of the order of 500-700° C. subatmospheric pressure and time of the order of 0.01 to 2 seconds to contact with a solid granular catalyst comprising essentially activated aluminum oxide which has relatively low catalytic activity supporting an oxide which has relatively high catalytic activity selected from the group consisting of the oxides of vanadium, columbium and tantalum.
5. A process for the dehydrogenation of paraffin hydrocarbons to produce diolefins therefrom, which comprises subjecting said paraffin hydrocarbons at a temperature of the order of 500-700° C. subatmospheric pressure and time

of the order of 0.01 to 2 seconds to contact with a solid granular catalyst comprising essentially a calcined aluminum hydrate of high adsorptive capacity supporting an oxide which has relatively high catalytic activity selected from the group consisting of the oxides of vanadium, columbium and tantalum.

6. A process for the dehydrogenation of aliphatic hydrocarbons to produce unsaturated derivatives thereof, which comprises subjecting said aliphatic hydrocarbons at a temperature of the order of 450-700° C., absolute pressure of the order of 0.25 to 7 atmospheres, and time from approximately 0.1 to 10 seconds to contact with a solid granular catalyst comprising essentially aluminum oxide which has a relatively low catalytic activity supporting vanadium oxide which has a relatively high catalytic activity.

7. A process for the dehydrogenation of aliphatic hydrocarbons to produce unsaturated derivatives thereof, which comprises subjecting said aliphatic hydrocarbons at a temperature of the order of 450-700° C., absolute pressure of the order of 0.25 to 7 atmospheres, and time from approximately 0.1 to 10 seconds to contact with a solid granular catalyst comprising essentially aluminum oxide which has a relatively low catalytic activity supporting columbium oxide which has a relatively high catalytic activity.

8. A process for the dehydrogenation of aliphatic hydrocarbons to produce unsaturated derivatives thereof, which comprises subjecting said aliphatic hydrocarbons at a temperature of the order of 450-700° C., absolute pressures of the order of 0.25 to 7 atmospheres, and time from approximately 0.1 to 10 seconds to contact with a solid granular catalyst comprising essentially aluminum oxide which has a relatively low catalytic activity supporting tantalum oxide which has a relatively high catalytic activity.

9. A process for the dehydrogenation of paraffin hydrocarbons to produce diolefins therefrom, which comprises subjecting said paraffin hydrocarbons at a temperature of the order of 500-700° C. subatmospheric pressure and time of the order of 0.01 to 2 seconds to contact with a solid granular catalyst comprising essentially

aluminum oxide which has relatively low catalytic activity supporting columbium oxide which has relatively high catalytic activity.

10. A process for the dehydrogenation of paraffin hydrocarbons to produce diolefins therefrom, which comprises subjecting said paraffin hydrocarbons at a temperature of the order of 500-700° C. subatmospheric pressure and time of the order of 0.01 to 2 seconds to contact with a solid granular catalyst comprising essentially aluminum oxide which has relatively low catalytic activity supporting tantalum oxide which has relatively high catalytic activity.

11. A process for dehydrogenating aliphatic hydrocarbons which comprises contacting the same under dehydrogenating conditions with an oxide of an element from the left-hand column of group 5 of the periodic table, supported on an activated alumina comprising a calcined aluminum hydrate of high adsorptive capacity.

12. A process for dehydrogenating aliphatic hydrocarbons having less than six carbon atoms in straight chain arrangement which comprises contacting the same under dehydrogenating conditions with an oxide of an element from the left-hand column of group 5 of the periodic table, supported on an activated alumina comprising a calcined aluminum hydrate of high adsorptive capacity.

13. A process for dehydrogenating paraffinic hydrocarbons which comprises contacting the same under dehydrogenating conditions with an oxide of an element from the left-hand column of group 5 of the periodic table, supported on an activated alumina comprising a calcined aluminum hydrate of high adsorptive capacity.

14. A process for converting normally gaseous paraffins to olefins which comprises contacting the paraffins under dehydrogenating conditions with an oxide of an element from the left-hand column of group 5 of the periodic table, supported on an activated alumina comprising a calcined aluminum hydrate of high adsorptive capacity.

JACQUE C. MORRELL.  
ARISTID V. GROSSE.